

1

3,627,545

BATH AND PROCESS FOR CHEMICAL  
METAL PLATING

Glenn O. Mallory, Jr., Inglewood, and Donald W. Baudrand, Temple City, Calif., assignors to Allied Research Products, Inc., Baltimore, Md.

No Drawing. Continuation of abandoned application Ser. No. 833,163, June 13, 1969, which is a continuation-in-part of application Ser. No. 804,369, Feb. 26, 1969, which is a continuation-in-part of abandoned application Ser. No. 661,218, Aug. 17, 1967, which in turn is a continuation-in-part of abandoned application Ser. No. 468,921, July 1, 1965. This application June 5, 1970, Ser. No. 41,784.

Int. Cl. C23c 3/02

U.S. Cl. 106—1

5 Claims

## ABSTRACT OF THE DISCLOSURE

A bath for plating a material with a transition metal selected from the class consisting of nickel, cobalt, iron and chromium by chemical deposition which comprises an aqueous solution of a coordination compound of the transition metal with a saturated short chain carboxylic acid having 1-6 carbon atoms and the hydroxy derivatives of the acid, a ligand complexing agent selected from the group of pyrophosphoric acid, ascorbic acid, erythorbic acid, the water-soluble salts thereof and their mixtures, and a transition metal reducing agent. The bath has a pH ranging from 1-14 and contains less than about 3400 p.p.m. of chloride and/or sulfate anions. When the material being plated is bismuth, cadmium, tin, lead or zinc, the bath contains less than 1000 p.p.m. of these anions.

This is a continuation of application Ser. No. 833,163, filed June 13, 1969, now abandoned, which in turn is a continuation-in-part of application Ser. No. 804,369, filed Feb. 26, 1969, which in turn is a continuation of Ser. No. 661,218, filed Aug. 17, 1967, now abandoned, which in turn is a continuation-in-part of application Ser. No. 468,921, filed July 1, 1965, now abandoned.

This invention relates to plating of a material by chemical deposition and, in particular, to the electroless plating of a metal selected from the group consisting of nickel, cobalt, iron, chromium and their mixtures on the surface of the material from an aqueous plating bath comprising a water-soluble source of the metal, a ligand complexing agent and a reducing agent.

The water soluble source of the metal is a coordination compound of the metal with a saturated short chain carboxylic acid having 1-6 carbon atoms and hydroxy derivatives of said acids. Representative monocarboxylic acids suitable for use in the present invention include formic and acetic acids; representative dicarboxylic acids include oxalic, malonic and succinic acids; suitable hydroxy carboxylic acids include glycolic, citric, lactic and gluconic acid.

The ligand complexing agent employed in the bath of this invention is one of the following compounds; pyrophosphoric acid, ascorbic acid, erythorbic acid, the water-soluble salts thereof and their mixtures.

Suitable reducing agents include hypophosphorous acid, an alkali, alkali metal or alkaline earth metal hypophosphite such as ammonium, sodium, potassium, lithium, calcium, magnesium, strontium, barium, etc. hypophosphites or various combinations thereof; water-soluble boranes such as dimethylamine borane and morpholine borane and hydrazine hydrates.

A buffering agent such as a weak acid or base can be employed to maintain the pH of the plating bath between 1 to 14 and the choice of the buffering agent will

2

depend upon whether an alkaline or acidic plating bath is to be employed. Representative buffering agents include sodium or potassium hydroxide and citric acid. For example, in a hypophosphite type bath, where the hardness of the metal plate is important, an acid bath is used since the greater amount of phosphorus deposited with the metal in an acid bath produces a substantially harder plate than an alkaline bath. Where the speed of plating is paramount, an alkaline bath is used. The higher plating rate of an alkaline bath prevents the deposition of amounts of phosphorus comparable to acid baths and the hardness of the plate is diminished.

Still other compounds can be included in the aqueous metal plating bath of this invention such as accelerating agents which include water soluble inorganic and organic carbonates. These accelerating agents also can function as secondary buffering agents and to some extent as complexing agents. Representative accelerating agents include ammonium, potassium, lithium, sodium and choline carbonate.

The aqueous plating bath of this invention thus comprises as a water-soluble source of the metal to be plated a coordination compound of nickel, cobalt, iron and chromium with a short chain carboxylic acid having 1-6 carbon atoms or the hydroxy derivatives thereof in amounts ranging from about 1-80 grams/liter; a ligand complexing agent selected from the group consisting of pyrophosphoric acid, ascorbic acid, erythorbic acid, the water-soluble salts thereof and their mixtures in amounts ranging from about 1-60 grams/liter; and a reducing agent in amounts ranging from about 1-100 grams/liter. The bath can also include a buffering agent in amounts sufficient to maintain the pH between 1-14 and generally amounts ranging from about 0.1-100 grams/liter will be sufficient to achieve this purpose. It will be recognized though that less or even greater amounts can be employed. If an accelerating agent is employed it can be added to the bath in amounts ranging from about 7.5-75 grams/liter.

In one embodiment of this invention the substrate plated with one or more of the above metals from a bath as described herein can be a substrate which the art recognizes as catalytic to the plating operation or one which can be plated through galvanic initiation or one which is rendered catalytic by sensitizing or pretreating the same. Thus the substrate can include such materials as iron, cobalt, nickel, ruthenium, rhodium, palladium, osmium, iridium, platinum, gold, copper, silver, beryllium, germanium, aluminum, carbon, vanadium, molybdenum, tungsten, chromium, selenium, titanium, uranium and plastics. In plating such a substrate the content of chloride and/or sulfate ions in the bath, in accordance with the present invention, is no greater than about 3400 p.p.m.

In another embodiment of the present invention the substrate plated with one or more of the above metals from a bath as described herein can be a non-catalytic substrate selected from the group consisting of bismuth, cadmium, tin, lead, zinc and their combinations. Heretofore it has been recognized in such publications as British Pat. 821,763 and U.S. Pat. 2,935,425 and 2,766,138 that conventional electroless plating solutions have been incapable of depositing plating metals on these materials. In plating such a substrate, the content of chloride and/or sulfate ions in the bath in accordance with the present invention is no greater than about 1000 p.p.m.

It has been known heretofore to produce electroless plating baths from a metal such as nickel, cobalt, iron or chromium in the form of its chloride, sulfate, formate, acetate, sulfonate, gluconate, succinate, malonate or citrate and to include in such a bath as a complexing agent various carboxylic and hydroxycarboxylic acids

such as citric, oxalic, tartaric, adipic, succinic, hydro-acetic, hydroxysuccinic, gluconic, hydroxymalonic and their water-soluble salts; various amines such as ethylene diamine, diethylene triamine, ethylene diamine tetra-acetic acid; and various short chain aliphatic aminocarboxylic acids such as  $\alpha$ -aminopropionic acid,  $\beta$ -aminopropionic acid, and  $\alpha$ -aminobutyric acid. Such disclosures can be found, for instance, in U.S. Pats. 2,871,142; 2,935,425; 2,942,990; 3,041,198; 3,096,182; 3,121,644; 3,148,072; 3,178,311 and 3,198,659.

The prior art has not recognized, however, that the liquid complexing agents of the present invention produce a bath exhibiting excellent stability characteristics when the bath is limited to a chloride and/or sulfate ion concentration of less than about 3400 p.p.m. and in the situation when a noncatalytic substrate of a metal selected from the group consisting of bismuth, cadmium, tin, lead, zinc or their combinations is to be plated, the chloride and/or sulfate ion concentration is less than about 1000 p.p.m.

It has been found that with plating baths including a chloride or sulfate ion concentration greater than the maximum values reported above, the stability of the bath is appreciably and deleteriously affected which in turn disadvantageously affects the plating rate and/or the quality of the plate deposited on a catalytic surface, notwithstanding the particular conventional complexing agent employed in combination therewith. In contrast, the present invention overcomes the instability of such plating baths by limiting the maximum concentration of sulfate and/or chloride ions therein and by incorporating with the heretofore defined water-soluble source of metal, specific ligand complexing agents. The present invention also provides a bath from which materials which heretofore were not considered to be platable from an electroless plating bath can be so plated.

The following examples illustrate the present invention when practiced to produce a coating of nickel, iron, cobalt or chromium, or combinations thereof on a catalytic surface from an acid or alkaline bath.

## EXAMPLE 1

|                                 | Preferred        | Range    |
|---------------------------------|------------------|----------|
| Nickel citrate, g.p.l.          | 34               | 16-60    |
| Potassium pyrophosphate, g.p.l. | 40               | 20-75    |
| Sodium hypophosphite, g.p.l.    | 25               | 10-100   |
| NaOH, ml.                       | ( <sup>1</sup> ) | 5-40     |
| pH                              | 9.5              | 9.0-11.0 |
| Temperature, ° F                | 140              | 80-200   |

<sup>1</sup> 20 ml. of conc. NH<sub>4</sub>OH per liter.

## EXAMPLE 2

|                                          | Preferred | Range    |
|------------------------------------------|-----------|----------|
| Cobaltous citrate, g.p.l.                | 25        | 15-40    |
| Sodium pyrophosphate, g.p.l.             | 35        | 10-80    |
| Sodium hypophosphite, g.p.l.             | 25        | 10-100   |
| Na <sub>2</sub> CO <sub>3</sub> , g.p.l. | 25        | 10-60    |
| pH                                       | 10.5      | 9.0-11.0 |
| Temperature, ° F                         | 160       | 130-212  |

## EXAMPLE 3

|                              | Preferred | Range   |
|------------------------------|-----------|---------|
| Ferrous gluconate, b.p.l.    | 50        | 35-65   |
| Sodium ascorbate, g.p.l.     | 15        | 5-30    |
| Dimethylamine borane, g.p.l. | 2         | 1-4     |
| Glucose, g.p.l.              | 10        | 3-30    |
| Potassium citrate, g.p.l.    | 30        | 10-80   |
| pH                           | 8.2       | 7.5-9.5 |
| Temperature, ° F             | 185       | 150-200 |

## EXAMPLE 4

|                                                          | Preferred | Range   |
|----------------------------------------------------------|-----------|---------|
| Chromous acetate, g.p.l.                                 | 25        | 15-40   |
| Sodium erythorbate, g.p.l.                               | 25        | 10-60   |
| Sodium hypophosphite, g.p.l.                             | 30        | 10-100  |
| (NH <sub>4</sub> ) <sub>2</sub> CO <sub>3</sub> , g.p.l. | 30        | 15-60   |
| pH                                                       | 8.1       | 7.5-9.8 |
| Temperature, ° F                                         | 175       | 150-200 |

## EXAMPLE 5

|                              | Preferred | Range    |
|------------------------------|-----------|----------|
| Nickel acetate, g.p.l.       | 12        | 6-30     |
| Cobaltous citrate, g.p.l.    | 25        | 10-60    |
| Sodium pyrophosphate, g.p.l. | 50        | 30-75    |
| Sodium hypophosphite, g.p.l. | 30        | 10-100   |
| Sodium carbonate, g.p.l.     | 25        | 10-40    |
| Sodium hydroxide, g.p.l.     | 5         | 1-10     |
| pH                           | 10.2      | 9.0-11.5 |
| Temperature, ° F             | 180       | 150-212  |

## EXAMPLE 6

|                           | Preferred | Range   |
|---------------------------|-----------|---------|
| Nickel glycolate, g.p.l.  | 30        | 15-50   |
| Morpholine borane, g.p.l. | 3         | 1-6     |
| Citric acid, g.p.l.       | 15        | 7.5-45  |
| pH                        | 2.4       | 1.0-7.0 |
| Temperature, ° F          | 100       | 60-200  |

Similar baths are prepared using as the source of the nickel, cobalt, iron, chromium or their mixtures the formates, acetates, oxalates, malonates, succinates, glycolates, citrates, lactates and gluconates thereof. Additionally, such baths can employ hypophosphorous acid or such hypophosphites as ammonium, lithium, calcium, magnesium and barium as the reducing agent.

In employing the above baths, conventional plating procedures are implemented. Thus, the temperature of the bath is adjusted to a suitable level ranging generally from ambient temperature to the boiling point of the bath. The material or article to be plated is placed in the bath and is retained therein until the metal in the desired thickness has been plated thereon.

The following examples illustrate a second embodiment of the present invention whereby it is now possible to plate such metals as cadmium, bismuth, tin, lead and zinc, although these materials heretofore were designated as non-catalytic materials which could not be plated electrolessly. For satisfactory plating it has been found that the amount of chloride and/or sulfate ions should be limited to an amount not in excess of 1000 parts per million of bath by weight.

## EXAMPLE 7

|                                        | Preferred | Range    |
|----------------------------------------|-----------|----------|
| Element:                               |           |          |
| Nickel ammonium glycolate, grams/liter | 40        | 15-60    |
| Ammonium hydroxide, percent by volume  | 15        | 10-20    |
| Sodium hydroxide, grams/liter          | 1         | 0.1-5    |
| Potassium carbonate, grams/liter       | 30        | 10-60    |
| Potassium pyrophosphate, grams/liter   | 30        | 15-60    |
| Sodium hypophosphite, grams/liter      | 18        | 10-60    |
| pH                                     | 9.7       | 8.9-11.0 |
| Temperature, ° F                       | 175       | 120-200  |

## EXAMPLE 8

|                                       | Preferred | Range    |
|---------------------------------------|-----------|----------|
| Element:                              |           |          |
| Nickel formate, grams/liter           | 25        | 15-60    |
| Ammonium hydroxide, percent by volume | 15        | 10-20    |
| Sodium hydroxide, grams/liter         | 1         | 0.1-5    |
| Potassium carbonate, grams/liter      | 30        | 10-60    |
| Potassium pyrophosphate, grams/liter  | 30        | 10-60    |
| Sodium hypophosphite, grams/liter     | 18        | 10-60    |
| pH                                    | 10.1      | 8.0-10.3 |
| Temperature, ° F                      | 150       | 120-200  |

## EXAMPLE 9

|                                      | Preferred | Range    |
|--------------------------------------|-----------|----------|
| Element:                             |           |          |
| Cobaltous glycolate, grams/liter     | 36        | 15-50    |
| Potassium citrate, grams/liter       | 40        | 20-100   |
| Potassium pyrophosphate, grams/liter | 30        | 7.5-60   |
| Sodium hydroxide, grams/liter        | 3         | 1-4      |
| Sodium hypophosphite, grams/liter    | 30        | 10-50    |
| pH                                   | 10.2      | 9.3-10.5 |
| Temperature, ° F                     | 150       | 65-180   |

## EXAMPLE 10

| Element:                                  | Preferred | Range    |
|-------------------------------------------|-----------|----------|
| Chromous acetate, grams/liter.....        | 20        | 10-25    |
| Potassium citrate, grams/liter.....       | 30        | 15-50    |
| Potassium pyrophosphate, grams/liter..... | 30        | 7.5-60   |
| Sodium erythorbate, grams/liter.....      | 15        | 3.0-25   |
| Sodium hypophosphite, grams/liter.....    | 20        | 10-50    |
| pH.....                                   | 9.5       | 9.1-10.3 |
| Temperature, ° F.....                     | 150       | 65-180   |

## EXAMPLE 11

|                                  | Preferred | Range   |
|----------------------------------|-----------|---------|
| Ferrous gluconate, g.p.l.....    | 50        | 25-75   |
| Sodium ascorbate, g.p.l.....     | 15        | 5-50    |
| Dimethylamine borane, g.p.l..... | 2         | 1-5     |
| Citric acid, g.p.l.....          | 20        | 10-100  |
| pH.....                          | 6.0       | 4.5-7.0 |
| Temperature, ° F.....            | 180       | 160-200 |

## EXAMPLE 12

|                                | Preferred | Range    |
|--------------------------------|-----------|----------|
| Nickel acetate, g.p.l.....     | 24        | 10-30    |
| Sodium erythorbate, g.p.l..... | 1.5       | 0.5-30   |
| Morpholine borane, g.p.l.....  | 3         | 1-6      |
| Ammonium hydroxide, g.p.l..... | (1)       | 5-30     |
| pH.....                        | 8.0       | 7.0-10.0 |
| Temperature, ° F.....          | 100       | 60-200   |

\* 10 ml. conc.

## EXAMPLE 13

|                                     | Preferred | Range    |
|-------------------------------------|-----------|----------|
| Nickel acetate, g.p.l.....          | 12        | 6-25     |
| Chromous acetate, g.p.l.....        | 12        | 6-25     |
| Potassium pyrophosphate, g.p.l..... | 40        | 30-80    |
| Potassium hypophosphite, g.p.l..... | 50        | 10-100   |
| KOH, g.p.l.....                     | 5         | 1-30     |
| pH.....                             | 10.1      | 8.0-12.5 |
| Temperature, ° F.....               | 180       | 160-212  |

Similar baths can be prepared using any of the sources of nickel, cobalt, iron and chromium defined above, alone or in combination. Further, the specific ligand complexing agent noted in each of the above baths can be replaced with any of the pyrophosphates, ascorbates or erythorbates identified herein.

The baths of the present invention provide a hard, bright, adherent plating not subject, to any substantial degree, to flaking or other deformation due to machining or fabricating of the plated material. In addition, the baths of this invention possess advantages such as greater ease and convenience of operation, operability at low

temperature if desired and enhanced stability characteristics and they provide increased plating rates.

What is claimed is:

1. A bath for plating a material selected from the group consisting of bismuth, cadmium, tin, lead and zinc with a transition metal selected from the class consisting of nickel, cobalt, iron and chromium by chemical deposition consisting essentially of an aqueous solution of
  - (a) a coordination compound of said transition metal with a saturated short chain mono- or dicarboxylic acid having 1-6 carbon atoms and the hydroxy derivatives of said acids, said coordination compound of said transition metal being present in an amount ranging between 1-80 grams/liter of said bath;
  - (b) a ligand complexing agent selected from the class consisting of ascorbic acid, erythorbic acid, the water-soluble salts thereof and their mixtures, said ligand complexing agent being present in amounts ranging between 1-60 grams/liter of said bath;
  - (c) a transition metal reducing agent selected from the group consisting of hypophosphorous acid, the alkali, alkali metal and alkaline earth metal salts thereof, dimethylamine borane, morpholine borane and hydrazine sulfate, said reducing agent being present in amounts ranging between 1-100 grams/liter; and
  - (d) a buffering agent in amounts sufficient to maintain the pH of the bath from about 1-14; said bath containing less than about 1000 p.p.m. of anions selected from the group consisting of chloride and sulfate anions or their mixtures.
2. The bath according to claim 1 wherein the saturated short chain monocarboxylic acid is formic or acetic acid.
3. The bath according to claim 1 wherein the saturated short chain dicarboxylic acid is oxalic, malonic or succinic acid.
4. The bath according to claim 1 wherein the hydroxy derivative of said acids is glycolic, citric, lactic or gluconic acid.
5. The bath according to claim 1 which includes 7.5-75 grams/liter of an accelerating agent selected from the class consisting of ammonium, potassium, lithium, sodium and choline carbonates.

## References Cited

## UNITED STATES PATENTS

- |           |        |              |
|-----------|--------|--------------|
| 3,041,198 | 6/1962 | Certa et al. |
| 3,096,182 | 7/1963 | Berzins.     |
| 3,178,311 | 4/1965 | Cann.        |

LORENZO B. HAYES, Primary Examiner

U.S. CL. X.R.

**Disclaimer**

3,627,545.—*Glenn O. Mallory, Jr.*, Inglewood, and *Donald W. Baudrand*, Temple City, Calif. BATH AND PROCESS FOR CHEMICAL METAL PLATING. Patent dated Dec. 14, 1971. Disclaimer filed Mar. 1, 1971, by the assignee, *Allied Research Products, Inc.*

Hereby disclaims the portion of the term of the patent subsequent to Aug. 3, 1988.

[*Official Gazette April 18, 1972.*]